

June 30, 1931.

J. A. CHRISTIE

1,812,285

GOLF BALL AND METHOD OF MANUFACTURING SAME

Filed Oct. 12, 1929



Fig. 1



Fig. 2



Fig. 3



Fig. 4



10

Fig. 5



10

Fig. 6



Fig. 7

INVENTOR

JOHN A. CHRISTIE

Ely & Barrow

BY

ATTORNEYS.

## UNITED STATES PATENT OFFICE

JOHN A. CHRISTIE, OF AKRON, OHIO

## GOLF BALL AND METHOD OF MANUFACTURING SAME

Application filed October 12, 1929. Serial No. 399,135.

This invention relates particularly to the manufacture of golf balls, although some aspects of the invention are not necessarily limited to the specific application to the game of golf. As the manufacture of golf balls is probably the field which affords the greatest and most profitable outlet for the invention and its widest use, it will be described for that purpose. It is to be understood, however, that should the invention be applicable to other fields, such fields are intended to be covered herein.

The satisfactory golf ball of the present time comprises a body or major portion composed of a thread or ribbon of rubber wound about a small rubber ball constituting a core under considerable tension, and enclosed within an outer gutta percha or hard rubber casing. This ball has up to the present time been the only satisfactory ball for the purpose, having the advantages of greatest resilience and consequently maximum flight. It is, however, expensive to manufacture, requiring special winding machinery to form the rubber body, and the outer covering is easily cut, thereby rendering the ball unplayable.

Attempts have been made prior to my invention to construct substitutes for the standard golf ball, but so far as I am aware, the resultant balls have not been satisfactory as they have not affected in any manner the dominating position of the standard wound ball.

The present invention, however, constitutes a method of manufacturing a ball which is equal in many respects to the standard golf ball, and in all other respects is superior thereto. The ball manufactured by the process disclosed is of equal resilience with the standard golf ball, and, therefore, has an equally long flight. It is cheaper to manufacture and will not cut under the most severe use. It is of the same weight for size as the standard golf ball, and gives the same "click" upon being struck which is recognized as characteristic of high grade golf balls. It does not get out of round and has the same characteristics in respect to its behavior on

the fairway and on the greens as the standard ball.

The best known method of manufacturing the improved golf ball will be described, reference being had to the accompanying drawings. It will be understood that while the description given herein is detailed so as to enable one skilled in the art to manufacture the improved article, such details need not necessarily be followed in every respect, but may be varied or modified within the scope of the invention as set forth herein and in the claims appended hereto.

In the drawings:

Figure 1 is a view showing the first step in the process, which comprises the milling and sheeting of the compound entering into the ball;

Figure 2 is a plan of a portion of one of the sheets illustrating the composition of the sheet;

Figure 3 is a view showing the next step in the process, which is the formation of a roll made from the sheet of Figures 1 and 2;

Figure 4 shows the dividing of the roll into individual masses or pellets for the making of individual balls;

Figure 5 shows the mass or pellets of Figure 4 in position in the mold;

Figure 6 is a view showing the ball within the mold, the mold being shown in section; and

Figure 7 is a cross-section through the finished ball on the line 7-7 of Figure 6.

In the manufacture of the ball of the present invention, a quantity of rubber is mixed with fibrous material, fillers, curing agents and a rapid accelerator so that the resultant product has the desirable qualities of weight, liveliness and toughness. For the rubber ingredient suitable raw rubber, preferably smoked sheets are used, although other grades of rubber standard upon the market may be employed. With this rubber is compounded a suitable quantity of filler or pigment, preferably china clay, although other fillers may be employed to give the ball its proper density and specific gravity. To assist in the vulcanization and also to provide additional

filler, zinc oxide or equivalent mineral substances may be employed.

To the rubber so compounded is added a suitable quantity of fibrous material, preferably cotton fibre, although silk fibre, wool, leather or asbestos may be used. Cotton fibre is preferred for its many desirable properties known to those skilled in this art.

Sulphur for vulcanization is also added together with an accelerator of the organic type which is used for obtaining a rapid vulcanization at high temperature. Many forms of accelerators are known and have been developed for this purpose. I have employed with success small portions of tetra-methyl-thiuram disulphide and di-ortho-tolyl-guanidine.

As an example merely, of a successful compound for the purpose, the following will suffice:

|                                 | Parts |
|---------------------------------|-------|
| Smoked sheets                   | 76    |
| Zinc oxide                      | 13    |
| China clay                      | 15    |
| 25 Cotton fibres                | 38    |
| Sulphur                         | 6     |
| Tetra-methyl-thiuram disulphide | 1     |
| Di-ortho-tolyl-guanidine        | 1     |
| 30                              | 150   |

These ingredients or any suitable substitute and equivalent thereof, are mixed in any suitable manner known to the trade, care being taken to avoid premature vulcanization owing to the presence of the powerful accelerating ingredients. The mass of rubber compounding ingredients is shown at 1 and is mixed and sheeted between rolls 2, which may be the usual mill rolls, being formed thereby into a thin sheet 3, the accelerator being added to the batch just before sheeting whereby there will be no substantial precurring in the thin sheet of stock produced. This sheet may be of any desired thickness, it being essential merely that there is no tendency to precurse and that in the subsequent rolling operation, no chamber or cavity be left at the center of the roll. For this purpose sheets of  $\frac{1}{2}$  of an inch have been successfully used, although such dimensions are not essential. Upon examination of the sheet, it will be found that the fibrous materials are evenly scattered and distributed throughout the sheet but are aligned more or less longitudinally of the sheet, the fibres being illustrated in Figures 2, 4 and 5 at 4.

The sheet is then rolled up into a very tight roll transversely of the direction in which it issued from the sheeting rollers without the presence of any crevices to trap air within the mass and the fibres 4 are thus aligned longitudinally of the cylinder thus formed.

The roll or cylinder is then cut into sections or pellets 8 along transverse lines 6,

each pellet being of sufficient size to completely fill a golf ball mold cavity, with little or no overflow. A pellet is then placed in a mold cavity 10, as shown in Figure 5, and the mold closed and subjected to vulcanizing temperatures under high pressure exerted upon the mold. It will be noted that by this method the molding pressure is applied in the direction in which the fibres are aligned in the stock, and consequently the fibres are buckled or crushed longitudinally thereof, knitting them together in the vulcanized ball in such a way that the ball will remain of true roundness upon removal from the mold. It has been discovered that if the mass is not subjected to pressure in this manner, the vulcanizing pressure serves only to temporarily hold the mass in true round form when in the mold, and upon removal there would be an internal readjustment of the fibres, resulting in the ball assuming an untrue shape. The mold may be cut to provide the mesh or dimpled surface standard in all golf balls.

As an example of the subsequent treatment, the holds may be subjected to a ten minute cure at 310° Fahrenheit. By the use of sulphur sufficient to vulcanize rubber to a comparatively hard state together with powerful accelerators and the higher temperatures for a short period, the finished ball, illustrated at 11 in Figure 7, is cured in a manner which is peculiar to this invention and gives the desirable attributes and properties to the finished ball. It will be found that while the rubber throughout the ball is completely vulcanized, the outer surface of the ball and to a short distance in the rubber is cured to such an extent as to be hard or substantially of the density and non-resilience of hard rubber or gutta percha, while the center of the ball is cured to a less extent, being highly resilient or elastic. This has been attempted to be illustrated in Figure 7 by showing the highly cured, hard outer shell or cover of the ball at 12 and the elastic, resilient interior of the ball which is more resilient at 14, that portion of the ball between the outer shell and the center gradually merging from the hard exterior to the yielding, resilient interior.

The hard exterior of the ball accords the non-cutting surface and gives the desirable click to the ball while the more resilient and less cured interior gives the ball its life and long flight. The fibres give the ball its resistance and assist in its valuable characteristics. The convolutions imparted to the ball during the winding process, which are illustrated in Figure 7, secure the proper balance and increase the life and elasticity of the ball. By reason of the alignment of the fibres longitudinally in the cylindrical masses from which the balls are formed and the placing of the masses in the molds, as

shown in Figure 5, it has been found that a ball of true roundness is secured, the fibres being crushed or buckled endwise by the molding pressure and having no tendency to expand the ball in any direction after the molding pressure is relieved.

What is claimed is:

1. The process of manufacturing golf balls or the like, comprising compounding rubber, fibres, a vulcanizing agent, and an active accelerator, sheeting the said compound, rolling up the sheet so obtained transversely of the direction in which it was sheeted, placing a charge of the rolled material in a mold, and curing under heat and pressure applied longitudinally of the roll of material for a short period at high temperature to obtain a ball, the outer shell of which is hard and highly cured, and the inner portion thereof less highly cured and more resilient.
2. The process of manufacturing golf balls or the like, comprising compounding rubber, a vulcanizing agent, and an active accelerator, sheeting the said compound, rolling a sheet so obtained into a tight cylinder, placing a section of the cylinder in a mold, and curing for a period sufficient to form a hard rubber outer shell with a softer rubber core.
3. That method of making golf balls or the like which comprises providing a mass of rubber containing fibres aligned more or less in one direction therein, and molding and vulcanizing said mass of rubber by heat and by application of pressure in said direction, whereby there will be no tendency in the completed ball for the fibres in the ball to readjust themselves upon release of the molding pressure so as to cause the ball to assume an untrue shape.
4. A golf ball of molded homogeneous rubber compound throughout, said compound including fibres and vulcanizing ingredients such as normally to vulcanize to hard state, the exterior portion of the ball being vulcanized to a comparatively hard state and the central portion of the ball being only partly vulcanized to a comparatively resilient or elastic state.
5. A golf ball composed entirely of a vulcanized homogeneous composition of rubber including a powerful accelerator and sulphur sufficient to produce hard rubber, said ball being vulcanized to a comparatively hard state at the surface and the center portion of the ball being only partly vulcanized to a comparatively resilient or elastic state.

JOHN A. CHRISTIE.